

May 14, 1940.

E. L. BARTHOLOMEW ET AL

2,200,765

HEAT TREATMENT OF CAST IRON

Filed May 13, 1937

2 Sheets-Sheet 1

A CAST IRON

Fig. 1



Fig. 2



INVENTORS

Edward L. Bartholomew  
John S. Paine Jr  
By their attorney  
Victor Cobb

May 14, 1940.

E. L. BARTHOLOMEW ET AL

2,200,765

HEAT TREATMENT OF CAST IRON

Filed May 13, 1937

2 Sheets-Sheet 2

B CAST IRON.

Fig. 3.



Fig. 4.



INVENTORS

Edward L. Bartholomew  
John L. Paine Jr  
By their Attorney  
Victor Gold

## UNITED STATES PATENT OFFICE

2,200,765

## HEAT TREATMENT OF CAST IRON

Edward L. Bartholomew and John D. Paine, Jr.,  
 Marblehead, Mass., assignors to United Shoe  
 Machinery Corporation, Borough of Flemington,  
 N. J., a corporation of New Jersey

Application May 13, 1937, Serial No. 142,446

4 Claims. (Cl. 148—21.7)

This invention relates to the heat treatment of ferrous material and is herein illustrated in connection with a method of heat treating cast iron in order to impart to it desired physical properties.

It is an object of our invention to provide a method of heat treating cast iron suitable, for example, for cams or other machine parts to produce structures which are especially resistant to wear. In carrying out the invention, iron castings are heated to a temperature above the critical range of the metal and are quenched at a temperature of from 350° F. to 750° F., the iron castings being maintained in a quenching bath for a period of about 15 to 30 minutes. It has been found that this treatment provides a product which is tough, relatively ductile, and which has comparatively high tensile strength. Cast iron treated in this manner has great wear resisting properties and is particularly adapted for use in cams, gears, and other machine parts which are subjected to rolling or sliding contacts. The excellent wear resisting properties are believed to result from the fact that the crystalline structure of such iron contains a considerable amount of retained austenite which is softer than, but much tougher and more ductile than, its decomposition products. When machine parts such as cams composed of this iron are run in, the ductility of the austenite permits such rearrangement and adjustment of the microscopic crystalline structure of the surface portions of the parts as is necessary to obtain well fitting smoothly operating machine elements. The running-in effects a cold-working operation of the material which breaks down the austenite into its decomposition products. The resulting structure is a finely divided crystalline aggregate containing one or more of the forms known as martensite, sorbite, eutectite, and pearlite, and is appreciably harder than before the cold working as well as being highly resistant to wear. Parts heat treated in the manner above set forth, when subjected to wear tests, have been found to stand up many times as long as similar parts machined as cast and heat treated in accordance with the methods heretofore employed.

In another aspect, the invention provides, as an article of manufacture, cast iron or iron castings, produced in accordance with the method above outlined, and having a crystalline structure which has the advantages enumerated above. The invention, in these and other aspects, is disclosed in the following specification which could be read in conjunction with the accom-

panying drawings, and is pointed out in the claims.

In the drawings:

Figs. 1 and 2 are diagrams illustrating the physical properties of one type of cast iron heat treated in accordance with the method of our invention; and

Figs. 3 and 4 are similar diagrams for another type of cast iron.

In carrying out the method we utilize iron which, as cast, contains 3.0% or more of carbon and which preferably contains also a small amount of nickel. Typical compositions of cast irons which may be employed are as follows:

|                 | Cast iron |         | 15 |
|-----------------|-----------|---------|----|
|                 | A         | B       |    |
| Silicon         | Percent   | Percent | 20 |
| Sulphur         | 1.42      | 1.24    |    |
| Manganese       | 0.117     | 0.130   |    |
| Phosphorus      | 0.37      | 0.44    |    |
| Total carbon    | 0.448     | 0.297   |    |
| Graphite        | 3.36      | 3.39    |    |
| Combined carbon | 2.50      | 2.50    |    |
| Nickel          | 0.86      | 0.89    | 25 |
| Chromium        | 1.52      | 1.44    |    |
| Iron            | Balance   | Balance |    |

The iron casting to be treated is heated above the critical range of the metal, that is, to a temperature above about 1375° F. and is maintained at that temperature for from about 15 to 30 minutes, depending upon the size of the casting, after which the casting is quenched in a salt or other suitable bath maintained at a temperature of from 350° to 750° F. for a period of from about fifteen to thirty minutes. The iron is then washed in boiling soda solution, and is permitted to cool to room temperature. A suitable bath may be composed of potassium nitrate, 53%, sodium nitrate, 7%, and sodium nitrite, 40%.

We have found that, in most instances, heating above the critical range to about 1550° F. for about 30 minutes gives satisfactory results for most castings of small or medium size, but that temperatures as high as 1700° F. may be employed effectively for large castings. Temperatures as low as about 1375° F. for periods as short as about 15 minutes may be employed for very small castings.

Heating above the critical range converts the iron of the untreated casting to its austenitic form which, upon quenching, decomposes into other crystalline forms, the amount of conversion of the austenite depending upon the temperature

30

35

40

45

50

55

of the quench and the length of time in the bath. The effect of the hot quench in the range of about 350° to 750° F. is to cause an appreciable amount of austenite to be retained, the amount retained varying from a low percentage at low temperatures of the bath to a high percentage at high temperatures of the bath. The presence of nickel is believed to assist materially in the retention of austenite, and cast irons containing from 1.0 to 2.5% nickel may be employed with good results.

The resulting hardness of the cast iron increases as the temperature of the bath is lowered, the Brinell hardness varying in treated irons of type "A" from about 240 up to about 480. This is illustrated by curves in Figs. 1 and 2 in which Brinell hardness numbers and tensile strength are plotted separately against quenching temperatures for a considerable number of heat treated specimens of 0.505 inch and 0.717 inch in diameter, respectively. Figs. 3 and 4 show similar curves for test specimens of type "B" iron. In type "B" irons the Brinell hardness after treatment varies from about 250 to 475.

Austenitic cast irons which have a Brinell hardness of over about 350 are exceedingly difficult to machine unless special tools are used. However, it is to be noted that for both type "A" and type "B" irons, a high tensile strength is obtained when the quenching temperature is in the neighborhood of 600° F. whereas the Brinell hardness is less than 350 and, consequently, the iron is machineable. In view of this, for many purposes, it has been found that the iron quenched in a bath of about 600° F. produces excellent results; that is, the iron, after being heat treated as cast, can be machined, no other heat treatment being required. With irons of a hardness of much over 350 it has been found expedient to machine the castings prior to the heat treatment. This has been done with satisfactory results since such castings have been found to have surprisingly little distortion as a result of the subsequent heat treatment.

The method above outlined is particularly advantageous when employed in connection with castings for cams or gears the surfaces of which, when in use, are subjected to rolling or sliding contact. When such cams or gears are run in it is found that the material lends itself readily to the fitting or running-in operation which effects a cold working of the material. At this time the material is tough and ductile, probably

due to its retained austenite, but during the cold working the austenite decomposes into a finely divided crystalline structure which is appreciably harder, and has a higher tensile strength than the material before being worked, and is well adapted to resist wear.

Having described our invention, what we claim as new and desire to secure by Letters Patent of the United States is:

1. The method of treating cast iron, containing over 3.0% carbon and from 1.0 to 2.5% nickel, so as to produce a machineable structure of comparatively high tensile strength, which comprises heating the iron to a temperature of about 1550° F., maintaining the iron at that temperature for 30 minutes, then quenching the iron in a bath maintained at about 600° F. for about 30 minutes, and cooling the iron to room temperature.

2. The method of treating cast iron containing 3.0 to 3.6% carbon, 1.0 to 2.5% silicon, 0.3 to 0.75% manganese, 0.07 to 0.15% sulphur, 1.0 to 2.5% nickel and 0.2 to 0.5% chromium, which comprises heating the iron to a temperature above its critical range for about 15 to 30 minutes, then quenching the iron in a bath maintained at a temperature of about 600° F. for about 15 to 30 minutes, and then cooling the iron to room temperature.

3. The method of treating cast iron containing 3.0 to 3.6% carbon, which comprises heating the iron to a temperature above its critical range for about 15 to 30 minutes, then quenching the iron in a bath maintained at a temperature of about 600° F. for about 15 to 30 minutes, and then cooling the iron to room temperature.

4. The method of treating cast iron castings containing at least 3.0% carbon to obtain a product having an appreciable amount of austenite retained therein so that upon cold working the austenite decomposes in a finely divided crystalline structure imparting hardness and resistance to wear to the product, which method comprises heating the castings to a temperature above its critical range for a period of time sufficient to provide a predominantly austenitic structure in the iron castings, then quenching the iron castings in a bath maintained at a temperature of from 550° F. to 750° F. for a period of from 15 to 30 minutes, and then cooling the iron to room temperature.

EDWARD L. BARTHOLOMEW.

JOHN D. PAINE, JR.